# EUROPEAN PATENT SPECIFICATION

(11) **EP 0 575 190 B1**
(45) Date of publication and mention of the grant of the patent: **17.09.1997**
(21) Application number: 93304762.3
(22) Date of filing: 17.06.1993
(51) Int. Cl.: H01F 1/153, H01F 3/00

(54) **Fe-base soft magnetic alloy and process for making same**
Weichmagnetische Legierung auf Eisenbasis und Herstellungsverfahren
Alliage magnétiquement doux à base de fer et procédé de fabrication

(30) Priority: 17.06.1992 JP 158338/92
(43) Date of publication of application: 22.12.1993
(73) Proprietor: MITSUI PETROCHEMICAL INDUSTRIES, LTD., Tokyo 100 (JP)
(72) Inventor: Watanabe, Hiroshi, c/o Mitsui Petrochem. Ind. Ltd., Sodegaura-shi, Chiba-ken (JP); Hirota, Yoshihiko, c/o Mitsui Petrochem. Ind. Ltd., Sodegaura-shi, Chiba-ken (JP)
(74) Representative: Cresswell, Thomas Anthony

(56) References cited:
- EP-A- 0 316 811
- JOURNAL OF APPLIED PHYSICS. vol. 70, no. 10 , 15 November 1991 , NEW YORK US pages 6241 - 6243 Y.FUJII ET AL
- PATENT ABSTRACTS OF JAPAN vol. 17, no. 67 (C-1025)10 February 1993 & JP-04 272 159 (SUMITOMO METAL IND)
- PATENT ABSTRACTS OF JAPAN vol. 17, no. 67 (C-1025)10 February 1993 & JP-04 272 159

## Description

### BACKGROUND OF THE INVENTION

### 1. Field of the Invention

The present invention relates to an Fe-based soft magnetic alloy and, in particular, to an alloy having excellent soft magnetic properties and a process for making it.

### 2. Description of the Related Art

Fe-based amorphous magnetic alloys having a high saturation magnetic flux density are known to be used as magnetic core materials for magnetic heads, high frequency transformers, saturable reactors, choke coils, etc. However, though Fe-based amorphous magnetic alloys are lower priced than Co-based ones, the former have the drawbacks of large core loss in the high frequency region and low permeability. In addition, it's saturation magnetostriction is high.

An Fe-B system alloy is known as a conventional Fe-system amorphous magnetic alloy. However, the alloys including B (boron) are highly priced because the element B is expensive.

One object of the present invention is to provide a novel Fe-based soft magnetic alloy, which can be substituted for the above-mentioned conventional soft magnetic materials and has a low saturation magnetostriction and a low iron loss.

Another object of the present invention is to provide an Fe-based soft magnetic alloy which is lower priced.

### SUMMARY OF THE INVENTION

Intense researche and studies of various Fe-base soft-magnetic alloys in view of the above objectives have revealed that addition of specific element(s) M, particularly Zr, to an Fe-P system Fe-based soft magnetic alloy can provide an improved Fe-based Fe-Si-B-Al soft magnetic alloy having excellent soft magnetic characteristics, for example, having an extremely low saturation magnetostriction, and that addition of Cu to the Fe-P-M system Fe-based soft magnetic alloy is effective for obtaining excellent soft magnetic properties of the resulting alloy. The present invention is based on these findings.

Specifically, there is provided in accordance with the present invention an Fe-based soft magnetic alloy which has a composition represented by the formula:

Fe_{100-a-b-c-d}PₐM_{b}M'_{c}Cu_{d}

where M is at least one element selected from the group consisting of Zr, Hf, Nb, Mo, W, Ta, Ti, V, Cr, Mn, Y and Ce;
M' is at least one element selected from the group consisting of Si, Al, Ga, Ge, Ru, Co, Ni, Sn, Sb and Pd;
a, b, c and d each are an atomic % (atom %) and
each satisfy 0 < a ≤ 25, 0 < b ≤ 15, 0 ≤ c ≤ 20, and 0 ≤ d ≤ 5. In particular, at least 30 % of the alloy structure is desired to be occupied by fine crystalline particles, and the crystalline particles are desired to be composed of bcc solid solution including mainly Fe.

### DETAILED DESCRIPTION OF THE INVENTION

P (phosphorous) is an essential element constituting the alloy of the present invention and addition of a determined amount of P (more than 0 atomic % and not more than 25 atomic %) enables the extension of the range of formation of amorphous alloys after quenching without using an expensive element B (boron). Thereby, the cost of preparation of the alloy can be reduced.

The content (a) of P is more than 0 atomic % and not more than 25 atomic %, preferably from 1 to 15 atomic %, more preferably from 2 to 12 atomic %.

The element(s) M added to the Fe-based soft magnetic alloy of the present invention is supposed to prevent crystallization of the Fe-P system crystal which hampers the soft magnetic properties of the alloy or to elevate its crystallization temperature. As mentioned M is at least one, i.e. one or more of the elements selected from the group consisting of Zr, Hf, Nb, Mo, W, Ta, Ti, V, Cr, Mn, Y and Ce. Particularly Zr is preferable. Addition of the element(s) M is further effective for making the crystal grain fine and for improving the ability of forming the amorphous phase of the alloy in the Fe-P system alloy.

The content (b) of the M element(s) is more than 0 atomic % and not more than 15 atomic %, preferably from 2 to 15 atomic %, more preferably from 3 to 12 atomic %.

The element(s) M' added to the Fe-based soft magnetic alloy of the pr-esent invention is one or more of the elements selected from the group consisting of Si, Al, Ga, Ge, Ru, Co, Ni,Sn, Sb and Pd. It is considered that these elements are dissolved in the Fe-based solid solution because they have a negative interaction parameter relative to Fe, that is, it is considered that the elements are described as being substituted for Fe atom in the α-Fe crystalline structure whereby stabilizing the bcc crystal. Thus, it is considered that the crystalline grain having a genuine magnetocrystalline anisotropy of bcc crystalline or low magnetostriction constant is formed to exhibit excellent soft magnetic properties.

The content (c) of the M' element(s) is from 0 atomic % to 20 atomic %, preferably from 1 to 15 atomic %.

Cu (copper) in the alloy of the present invention is effective for making the crystalline particles obtained by the heat-treatment of the amorphous fine. Further, it improves the magnetic properties of the alloy since the effective magnetic anisotropy energy becomes smaller than its genuine magnetocrystalline anisotropy energy as the particles become fine. However, the copper content should not be more than 5 atomic % with respect to the preparation of the alloy because the just quenched alloy tends to be brittle. Accordingly, the content (d) of Cu is from 0 to 5 atomic %, preferably from 0.5 to 3 atomic %.

Incidentally, alloy further containing inevitable impurities such as N, S, O etc., to the extent that these elements do not deteriorate the properties of the alloy, is also included in the scope of the present invention .

The Fe-based soft magnetic alloy according to the present invention has an alloy structure, at least 30 % (30 % - 100 %) of which consists of (is composed of) fine crystalline particles, with the balance of the structure being an amorphous phase or other crystals than above-mentioned fine crystalline particles. The range of the ratio of the fine crystalline particles in the structure provides the alloy with excellent (soft) magnetic properties. In the present invention, even if the crystalline particles occupy substantially 100 % of the structure, the alloy retains sufficiently good magnetic properties. Preferably at least 50 %, more preferably 70 % or more of the alloy structure consists of (is composed of) the fine crystalline particles in view of magnetic properties.

The crystalline particles of the alloy of the present invention has mainly a bcc structure and it is considered that Fe is the main component in which M, M' and a small amount of P are believed to be dissolved.

It is preferred that the crystalline particles to be formed in the alloy of the present invention have a particle size of 1000 Å or less, preferably 500 Å or less, more preferably 50 to 300 Å. The particle size being 1000 Å or less, preferably 500 Å or less, more preferably 50 to 300 Å, provides the alloy of the present invention having excellent magnetic properties.

Preferred Fe-based soft magnetic alloys of the present invention have a saturation magnetostriction (λS) in the range of +10x10⁻⁶ to -5x10⁻⁶.

The proportion of the crystalline grains to the total alloy structure in the alloy of the present invention may be determined experimentally by an X-ray diffraction method or the like. Briefly, on the basis of the standard value of the X-ray diffraction intensity of Fe-based crystal in the completely crystallized condition (saturated X-ray diffraction intensity condition), the proportion of the X-ray diffraction intensity of the magnetic alloy material sample to be examined to the standard value may be obtained experimentally.

The average size of the crystalline particles is determined from Scheller's equation (t=0.9λ/β·cosθ) by using bcc peak reflection of the X-ray diffraction pattern (Element of X-ray Diffraction (Second Edition), pages 91-94, B.D. Cullity).

The Fe-based soft magnetic alloy of the present invention may be produced by a heat-treatment of an amorphous metal having a determined shape which is obtained by a common method of forming an amorphous metal. For instance, an amorphous alloy is first formed in the form of a ribbon, powder, fiber, or thin film by a melt quenching method such as a single roll method or double roll method, a thin film forming method such as a cavitation method, sputtering method or vapor deposition method, or a powder forming method such as mechanical alloying or the like. The resulting amorphous alloy is optionally shaped and worked into a desired shape, then it is heat-treated so that at least a part, preferably 30 % or more of the whole, of the sample is crystallized to obtain the alloy of the present invention.

The structure of the alloy after rapid-quenching is preferably amorphous but it may include partial crystalization to the extent that the resulting alloy exhibits soft magnetic properties after heat-treatment.

Generally, a quenched alloy ribbon is formed by a single roll method, and this is shaped into a determined shape such as a coiled magnetic core and then heat-treated. The heat-treatment is effected in vacuum, in an inert gas atmosphere, such as an argon gas or nitrogen gas atmosphere, in a reducing gas atmosphere such as H₂ or in an oxidizing gas atmosphere such as air. Preferably, it is carried out in vacuum or in an inert gas atmosphere. The heat-treatment temperature is approximately from 200 to 800°C, preferably approximately from 300 to 700°C, preferably from 350 to 700°C and more preferably from 400 to 700 °C. The heat-treatment time is within 24 hours, preferably about from 0.5 to 5 hours. The heat-treatment may be effected either in the absence or presence of a magnetic field. Impressing of a magnetic field brings a magnetic anisotropy to the alloy.

By the heat treatment of the amorphous alloy being carried out in the aforementioned range of temperatures and within the aforementioned time range, a soft magnetic alloy having excellent properties is obtained.

### BRIEF DESCRIPTION OF THE DRAWING

Fig. 1 is a graph showing X-ray diffraction patterns of the Fe-base soft magnetic alloy of the present invention after heat-treatment.

### EXAMPLES

Examples of the present invention are described hereinafter.

### Examples 1-3

A quenched ribbon (thin film) sample having a width of about 1.5 mm and a thickness of about 15-24 µm was formed from a melt containing Fe, P, Zr, and (Cu) in an argon gas atmosphere of one atmosphere pressure by a single roll method. The sample was then heat-treated at the temperature shown by Table 1 for about one hour in the presence of a nitrogen gas and in the absence of a magnetic field.

The iron loss (Pc W/kg) of each of the samples was determined under the condition of a frequency of 100 kHz and a maximum magnetic flux density of 0.1 T. The permeability (µ) (1KHz) under the condition of a frequency of 1 kHz and a maximum exciting magnetic field of 5 mOe, the saturation magnetization Ms (emu/g) and the saturation magnetostriction constant λs (×10⁻⁶) of each samples were also determined. The composition of the alloy samples, the content of the fine crystalline particles in the alloy and the average particle size are shown in Table 1 below.

**Table 1**

| | Composition of Alloy (atomic %) | Temperature of heat-treatment(°C) | Content of crystalline particle(%) | Particle size of Crystal (Å) |
|---|---|---|---|---|
| Exam.1 | Fe₈₉Zr₉P₂ | 620 | 60 or more | - |
| Exam.2 | Fe₈₅Zr₉P₆ | 620 | 60 or more | - |
| Exam.3 | Fe₈₈Zr₉P₂Cu₁ | 620 | 60 or more | 170 |
| Comp. Exam. | Fe₇₈Si₉B₁₃ | 410 | - | - |

As shown by Table 1, the content of the fine crystalline particles is 60 % or more in all of the samples. The composition of the alloy was determined by IPC analysis.

The magnetic properties are shown in Table 2.

As comparative samples, a rapid quenched alloy of Fe₇₈Si₉B₁₃ (Comparative Example, commercial product) was prepared as in the same condition as the example 1, and the iron loss, permeability, saturation magnetization and saturation magnetostriction of these samples were also shown in Table 2 below.

**Table 2**

| | Iron Loss (Pc.CW/kg) | Permeability (µ, 1kHz) | Saturation Magnetization (Ms,emu/g) | Saturation Magnetostrication (×10⁻⁶) |
|---|---|---|---|---|
| Exam.1 | 50 | 3400 | - | - |
| Exam.2 | 35 | 4700 | - | - |
| Exam.3 | 30 | 8000 | - | -0.6 |
| Comp. Exam. | 40 | 5600 | 170 | 28 |

As is obvious from the results in Table 2 above, the iron loss and the permeability of the alloy samples of the present invention are almost the same as those of the sample of Comparative Example and the alloy of the present invention is found to be sufficiently practical for the magnetic material substituted for the Fe-B amorphous soft magnetic alloy.

Fig. 1 shows the X-ray diffraction curves of the alloy of Fe₈₈Zr₉P₂Cu₁ (atomic %)(Example 3) obtained by heat-treating the quenched alloy formed by a single roll method, at 620 °C in the presense of argon for one hour. As is obvious from the figure, the structure of the alloy obtained by heat-treatment has mainly bcc structure.

As is obvious from the results in the above-mentioned examples, the Fe-based soft magnetic alloy of the present invention shows an excellent magnetic properties such as low ion loss, high permeability and low saturation magnetostriction by adding specific element(s), particularly Zr together with Cu to Fe-P system alloy. Accordingly, the alloy of the present invention can be utilized widely for a magnetic head, high-frequency transformers, saturable reactors, choke coils and like as the magnetic material substitited for the Fe-B system soft magnetic alloy.

In addition, the Fe-based soft magnetic alloy of the present invention can be prepared at a reduced cost since it utilizes phosphorous P instead of boron B.

## Claims

1. An Fe-based soft magnetic alloy having a composition of formula:${\text{Fe}}_{\text{100-a-b-c-d}} {\text{P}}_{\text{a}} {\text{M}}_{\text{b}} {\text{M'}}_{\text{c}} {\text{Cu}}_{\text{d}}$ where
M is at least one element seleted from Zr, Hf, Nb, Mo, W, Ta, Ti, V, Cr, Mn, Y and Ce; M' is at least one element selected from Si, Al, Ga, Ge, Ru, Co, Ni, Sn, Sb and Pd;
a, b, c and d each are an atomic % and satisfy the relations: 0 < a ≤ 25, 0 < b ≤ 15, 0 ≤ c ≤ 20, and 0 ≤ d ≤ 5.

2. An alloy according to claim 1 in which at least 30% of the alloy structure is occupied by fine crystalline particles.

3. An alloy acording to claim 2 in which the crystalline particle is a bcc solid solution including mainly iron.

4. An alloy according to any one of claims 1 to 3 in which the average size of the particles is not more than 100nm.

5. An alloy according to any one of claims 1 to 4 in which the saturation magnetostriction (λs) of the alloy is from +10 x 10⁻⁶ to -5 x 10⁻⁶.

6. A process for making an Fe-based soft magnetic alloy comprising
forming a quenched alloy having a composition of formula${\text{Fe}}_{\text{100-a-b-c-d}} {\text{P}}_{\text{a}} {\text{M}}_{\text{b}} {\text{M'}}_{\text{c}} {\text{Cu}}_{\text{d}}$ wherein
M is at least one element selected from Zr, Hf, Nb, Mo, W, Ta, Ti, V, Cr, Mn, Y and Ce; M' is at least one element selected from Si, Al, Ga, Ge, Ru, Co, Ni, Sn, Sb and Pd; a, b, c and d each are an atomic % and each satisfy the relations
0 < a ≤ 25, 0 < b ≤ 15, 0 ≤ c ≤ 20, and 0 ≤ d ≤ 5,
by a melt quenching method, a thin film forming method or a powder forming method and treating the quenched alloy by heat.

7. A process according to claim 6 in which the quenched alloy is maintained at the temperature from 350 °C to 700 °C for less than 24 hours during heat-treatment.

8. A process according to claim 6 or claim 7 for producing an alloy according to any one of claims 2 to 5.

9. A magnetic core consisting of an alloy according to any one of claims 1 to 5 or produced according to claim 6 or claim 7.

## Patentansprüche

1. Weichmagnetische Legierung auf Fe-Basis mit einer Zusammensetzung der Formel:${\text{Fe}}_{\text{100-a-b-c-d}} {\text{P}}_{\text{a}} {\text{M}}_{\text{b}} {\text{M'}}_{\text{c}} {\text{Cu}}_{\text{d}} \text{,}$ in der M mindestens ein Element ist, ausgewählt aus Zr, Hf, Nb, Mo, W, Ta, Ti, V, Cr, Mn, Y und Ce, M' mindestens ein Element ist, ausgewählt aus Si, Al, Ga, Ge, Ru, Co, Ni, Sn, Sb und Pd, a, b, c und d jeweils Atom-% sind und den folgenden Beziehungen entsprechen: 0 < a ≤ 25, 0 < b ≤ 15, 0 ≤ c ≤ 20 und 0 ≤ d ≤ 5.

2. Legierung nach Anspruch 1, wobei mindestens 30 % der Struktur der Legierung von feinen kristallinen Teilchen eingenommen werden.

3. Legierung nach Anspruch 2, wobei die kristallinen Teilchen eine feste bbc-Lösung sind, enthaltend hauptsächlich Eisen.

4. Legierung nach einem der Ansprüche 1 bis 3, wobei die mittlere Teilchengröße nicht mehr als 100 nm beträgt.

5. Legierung nach einem der Ansprüche 1 bis 4, wobei die Sättigungsmagnetostriktion (λs) der Legierung +10 x 10⁻⁶ bis -5 x 10⁻⁶ ist.

6. Verfahren zur Herstellung einer weichmagnetischen Legierung auf Fe-Basis, umfassend
Bildung einer abgeschreckten Legierung mit einer Zusammensetzung der Formel${\text{Fe}}_{\text{100-a-b-c-d}} {\text{P}}_{\text{a}} {\text{M}}_{\text{b}} {\text{M'}}_{\text{c}} {\text{Cu}}_{\text{d}} \text{,}$ in der M mindestens ein Element ist, ausgewählt aus Zr, Hf, Nb, Mo, W, Ta, Ti, V, Cr, Mn, Y und Ce, M' mindestens ein Element ist, ausgewählt aus Si, Al, Ga, Ge, Ru, Co, Ni, Sn, Sb und Pd, a, b, c und d jeweils Atom-% sind und den folgenden Beziehungen entsprechen: 0 < a ≤ 25, 0 < b ≤ 15, 0 ≤ c ≤ 20 und 0 ≤ d ≤ 5,
durch ein Schmelz/Abschreck-Verfahren, ein Verfahren zur Erzeugung eines dünnen Films oder ein Verfahren zur Erzeugung eines Pulvers und Behandeln der abgeschreckten Legierung durch Wärme.

7. Verfahren nach Anspruch 6, wobei die abgeschreckte Legierung während der Wärmebehandlung weniger als 24 Stunden bei einer Temperatur von 350 bis 700°C gehalten wird.

8. Verfahren nach Anspruch 6 oder 7 zur Herstellung einer Legierung nach einem der Ansprüche 2 bis 5.

9. Magnetischer Kern, bestehend.aus einer Legierung nach einem der Ansprüche 1 bis 5 oder hergestellt nach Anspruch 6 oder 7.

## Revendications

1. Alliage magnétique doux à base de fer, qui présente une composition répondant à la formule :${\text{Fe}}_{\text{(100-a-b-c-d)}} {\text{P}}_{\text{a}} {\text{M}}_{\text{b}} {\text{M'}}_{\text{c}} {\text{Cu}}_{\text{d}}$ dans laquelle M représente au moins un élément choisi parmi Zr, Hf, Nb, Mo, W, Ta, Ti, V, Cr, Mn, Y et Ce ; M' représente au moins un élément choisi parmi Si, Al, Ga, Ge, Ru, Co, Ni, Sn, Sb et Pd ; a, b, c et d représentent chacun un pourcentage atomique et satisfont aux relations 0 < a ≤ 25, 0 < b ≤ 15, 0 ≤ c ≤ 20 et 0 ≤ d ≤ 5.

2. Alliage conforme à la revendication 1, dans lequel au moins 30 % de la structure d'alliage est occupée par des particules fines cristallines.

3. Alliage conforme à la revendication 2, dans lequel les particules cristallines se trouvent dans une solution solide de structure cubique centrée (cc) comprenant principalement du fer.

4. Alliage conforme à l'une quelconque des revendications 1 à 3, dans lequel la taille moyenne des particules ne dépasse pas 100 nm.

5. Alliage conforme à l'une quelconque des revendications 1 à 4, dans lequel le coefficient de magnétostriction à saturation (λs) de l'alliage est comprise entre +10 x 10⁻⁶ et -5 x 10⁻⁶.

6. Procédé de fabrication d'un alliage magnétique doux à base de fer, comprenant :
la mise en forme d'un alliage trempé qui présente une composition répondant à la formule :${\text{Fe}}_{\text{(100-a-b-c-d}} {\text{)P}}_{\text{a}} {\text{M}}_{\text{b}} {\text{M'}}_{\text{c}} {\text{Cu}}_{\text{d}}$ dans laquelle M représente au moins un élément choisi parmi Zr, Hf, Nb, Mo, W, Ta, Ti, V, Cr, Mn, Y et Ce ; M' représente au moins un élément choisi parmi Si, Al, Ga, Ge, Ru, Co, Ni, Sn, Sb et Pd ; a, b, c et d représentent chacun un pourcentage atomique et satisfont chacun aux relations 0 < a ≤ 25, 0 < b ≤ 15, 0 ≤ c ≤ 20 et 0 ≤ d ≤ 5,
par un procédé de trempe à l'état fondu, un procédé de mise sous forme de film mince ou un procédé de mise sous forme de poudre, et le traitement thermique de l'alliage trempé.

7. Procédé conforme à la revendication 6, dans lequel l'alliage trempé est maintenu à une température comprise entre 350° C et 700° C pendant moins de 24 heures au cours du traitement thermique.

8. Procédé conforme à la revendication 6 ou 7 pour produire un alliage conforme à l'une quelconque des revendications 2 à 5.

9. Noyau magnétique constitué d'un alliage conforme à l'une quelconque des revendications 1 à 5, ou produit selon la revendication 6 ou 7.
